

Dec. 22, 1931.

E. F. KENNEY

1,837,189

RAIL HEAT TREATMENT

Filed April 29, 1931



Inventor

*Edward F. Kenney.*

By *R. S. C. Daugherty.*  
Attorney

## UNITED STATES PATENT OFFICE

EDWARD F. KENNEY, OF BETHLEHEM, PENNSYLVANIA, ASSIGNOR TO BETHLEHEM STEEL COMPANY, A CORPORATION OF PENNSYLVANIA

## RAIL HEAT TREATMENT

Application filed April 29, 1931. Serial No. 533,791.

My invention relates to the heat treatment of rails and other massive bodies. This application is a continuation in part of application Serial No. 377,780, filed July 12, 1929.

An important object of my invention is the prevention of permanent strains in the metal of rail or other massive body which tend to be produced therein during cooling, particularly during such rapid cooling as occurs during quenching.

When a rail is subjected to a rapid cooling operation, marked temperature differentials are produced between different portions of the rail metal. These differentials of temperature, particularly those between the interior and exterior portions of the head, produce more or less severe strains in the metal, which may result in permanent weaknesses or other defects in the rail, if the rail is allowed to cool in the usual way. It is an important purpose of my invention to prevent these strains from resulting in permanent defects in the metal. Accordingly, a significant feature of my invention is the elimination of these strains while the rail is still hot. This I accomplish by subjecting the rail, while in its condition of having marked temperature differentials, to a rapid heating operation to quickly reduce the temperature differentials.

To illustrate my invention a specific embodiment thereof will now be described. The drawing gives a cross section, full sized, of a rail to which this specific description applies. This rail weighs about 130 lbs. per yard, is thirty-nine feet long, and has a composition within the following ranges:

|  | Carbon | Manganese | Phosphorus | Sulphur | Silicon |
|--|--------|-----------|------------|---------|---------|
|  | .62    | 1.32      | .023       | .044    | .16     |
|  | .72    | 1.43      | .022       | .042    | .19     |
|  | .68    | .72       | .023       | .062    | .13     |
|  | .72    | .79       | .024       | .060    | .19     |
|  | .74    | .69       | .023       | .049    | .26     |
|  | .86    | .81       | .023       | .057    | .22     |

A rail of the cross section shown is produced in the rail mill in the usual way. The rail is allowed to cool from the mill heat until an edge of one of the flanges becomes mag-

netic. Obviously, at this stage, by far the greater mass of the rail is still above the critical range. In this state the rail is immersed in a water bath for 30 seconds and is then removed and immediately transferred to and immersed in a bath of molten lead having a temperature of about 1000° F. It is kept in this lead bath a period of from 4 to 5 minutes. From the lead bath it is immediately transferred to a closed furnace which is maintained at a temperature of about 1000° F. where it is kept at substantially a uniform temperature for a period preferably of between one hour and one and one-half hours, although it may be kept in this furnace a somewhat greater length of time, say up to three hours. The rail is then withdrawn from the furnace and allowed to cool in the air.

The treatment of the rail just outlined comprises first, rapidly cooling the greater part of the rail metal through the critical range; second, the rapid reduction of temperature differentials in the rail in the lead bath, which differentials have been produced by the rapid cooling operation; third, drawing the metal of the rail in the furnace, that is to say, producing a sorbitic or troostite-sorbitic micro-structure in the hardened metal; and fourth, cooling the rail to atmospheric temperatures.

The rapid cooling of the rail metal occurs not only while the rail is actually in the aqueous quenching bath but continues through the interval which elapses between the removal from the water bath and the immersion in the lead bath. While the immersion in the lead bath "immediately" follows the removal from the water bath it will be obvious that in handling an object such as a rail the time interval between the two steps must necessarily be of appreciable duration. In treating full sized rails of the section shown I have ordinarily kept this time interval at twenty seconds or less. It is well to bear in mind, however, that the rapid cooling operation continues for a short interval after the removal from the actual quenching bath.

This step of rapidly cooling the rail pro-

duces very marked differences of temperature in different parts of the rail. The thinner parts, as the web and flanges, will be at substantially lower temperatures than the head; the exterior portions of the rail will be at much lower temperatures than the interior. These temperature differentials of interior and exterior portions are especially pronounced in the head. Consequently the immediate immersion of the rail in a lead bath at 1000° F. is especially important in preventing permanent strains and allied defects from being produced in the rail head. Upon immersion in the lead bath at 1000° F. heat energy is rapidly communicated to the exterior of the rail and the temperature differentials are rapidly reduced.

When the rail is immersed in the lead bath a goodly proportion of the rail mass is still above the blue heat zone. Particularly is this true of the head. While the rapid cooling operation has been sufficient to lower the temperature of the entire mass of rail metal to temperatures below the critical range, the interior of the head is still above the blue heat zone. This is important as the elimination or substantial reduction of temperature differentials in the head while a considerable mass thereof is still above the blue heat zone greatly diminishes the chances of permanent defects from the strains produced by temperature differentials. Four to five minutes in the lead bath for this particular section of rail, cooled as above, is sufficient to substantially equalize the temperatures of the rail.

As above indicated, the rail is next taken from the lead bath to a furnace maintained at about 1000° F. for "drawing" the metal of the rail which has passed rapidly through the critical range, with the resulting transformation of the micro-structure of this metal to the sorbitic or troostite-sorbitic state. Following this the rail is allowed to cool in the air.

A modification of the process just outlined has been very successful. Following a quench in water for 30 seconds, as in the previous example, the rail is immersed in a lead bath having a temperature of 850 to 875° F. for three minutes, and then immediately transferred to the "drawing" furnace having a temperature of 850° to 875° F. in which it is held for 1½ hours. By using lower temperatures than in the previous example substantially higher mechanical properties such as tensile strength and elastic limit are secured.

In these two illustrations of the invention the temperatures employed for the lead bath and the durations of immersion therein are sufficient to effect substantial equalization of the temperatures of the rail. While substantial equalization is desired, successful re-

sults may also be obtained where complete uniformity of temperature is not secured. For example, following the quench, the rail may be immersed in a lead bath having a temperature of 800° F. for one minute. Following this treatment there will still be appreciable differences of temperature between portions of the rail but they will be so reduced that equalization of temperature will be quickly accomplished when the rail is placed in the drawing furnace. The primary function of the lead bath is to quickly reduce the temperature differences in the rail, whether such reduction of temperature differences is carried to a condition of temperature uniformity or not.

The process just described may be modified by effecting the drawing operation in the lead bath instead of in the furnace. Instead of keeping the rail in a lead bath just long enough to reduce temperature differentials, as in the process just described, the immersion in the lead bath is prolonged sufficiently to effect the drawing operation. Instead of an immersion in the lead bath for a period of from four to five minutes, the immersion will be maintained for one hour or longer. After withdrawal from the lead bath the rail is allowed to cool in the air.

Obviously the time periods given for rapid cooling, lead bath treatment, and drawing will vary somewhat with the particular section and weights of metal treated. The figures given have been found to be effective with the particular section shown.

The best results have been obtained when the entire mass of the rail head has been rapidly cooled through the critical range but obviously my process is not limited to such treatment. For example, the rapid cooling operation may be so limited in duration that a substantial portion of the interior of the rail head is not rapidly cooled through the critical range, and only a portion of the head metal therefore being hardened.

Obviously the process may be altered in various ways. For example, instead of cooling from the mill heat until an edge of the flange becomes magnetic and then quenching, as above given, the rail may be equalized at a definite temperature above the critical range and then quenched.

Although it is advantageous to quench from the mill heat, whether or not an equalizing operation is employed prior to the quench, it may be desirable at times to reheat and treat rails which have already been cooled to atmospheric temperatures. Obviously in such case the rail may be heated above the critical range and then treated in accordance with the methods already outlined.

In several of the claims which follow reference is made to the head only of the rail, the other parts of the rail not being men-

tioned. Obviously such claims are not intended to be limited to methods in which the head alone is treated. These claims specify the head because of the fact that this portion of the rail is the most important as regards my treatment and the process is effective whether or not the other parts of the rail are treated. Obviously it is correct to refer to the head having been subjected to the steps of my process whether or not the remaining parts of the rail have been also subjected thereto.

Instead of a lead bath for quickly reducing temperature differences other liquid baths may be successfully employed. For example I have found certain salt baths to be successful. As an illustration mention may be made of a salt bath made of equal weights of sodium nitrate and potassium nitrate. The mixture of the two nitrates is fused and the temperature of the resulting bath maintained at a temperature say of 850 to 875° F. The rail is immersed in this bath, as in the lead bath, to reduce or eliminate temperature differences. Ordinarily the use of this bath requires a longer immersion than the lead bath. I have found a 50% increase in time to be suitable. To effect a substantial uniformity of temperature of the rail before it is placed in the drawing furnace and when the temperature of the salt bath is 875° F. about five to six minutes is sufficient.

As is evident from the illustrative embodiments of the invention given above the temperatures of the liquid bath may vary considerably. Preferably the temperatures of such bath should not be below the blue heat zone.

What I desire to emphasize in this connection is that the important thing is to rapidly transfer heat to the rail to quickly reduce temperature differences and this may be effected in a metal bath, as lead, or in some other fluid material as for example various salt mixtures.

What I mean by the "blue-heat zone", as this expression is used in this disclosure, is that range of temperatures, below the critical range where steels in heating increase in tensile strength and the elastic limit, and also decrease in ductility. At temperatures, within this range, most steels when exposed to air take on a blue color, due to oxidation, but since, with some steels, this color is not readily apparent, I do not wish to be limited to the color as a means of determining or defining this zone.

By the expression "critical range" I mean that temperature range through which the steel must be cooled to effect a hardening thereof.

Having thus described my invention what I claim as new and desire to secure by Letters Patent is:

1. In a process for the treatment of rails, the steps of rapidly cooling a rail to cause a substantial portion of at least the head of the rail to pass rapidly through the critical range, and then immersing the rail while still hot in a liquid bath maintained at a temperature not lower than the blue heat zone to rapidly reduce the temperature differentials in the rail.

2. In a process for the heat treatment of rails, the steps of immersing a rail, the major portion of at least the head of which is above the critical range, in an aqueous bath for a sufficient time to rapidly cool a substantial portion of the head through the critical range, withdrawing from the aqueous bath, and then before the innermost portions of the head have reached the blue heat zone immersing the rail in a liquid bath maintained at a temperature not lower than the blue heat zone to quickly reduce temperature differentials.

3. In a process for the treatment of rails, the steps of rapidly cooling a rail and then, while the innermost portions of the head of the rail are still above the blue heat zone, subjecting the rail to a hot liquid metal of high specific gravity to quickly reduce the temperature differentials.

4. In a process for the treatment of rails, the steps of rapidly cooling the rail, a substantial proportion of at least the head of the rail being passed rapidly through the critical range, immersing the rail while still hot in a liquid bath maintained at a temperature not lower than the blue heat zone to rapidly reduce the temperature differentials in the rail and then subjecting the rails to a drawing operation in a furnace.

5. In a process for the treatment of rails, the steps of rapidly cooling a rail whereby marked temperature differentials are produced and then immersing the rail while still hot in a liquid bath maintained at a temperature not lower than the blue heat zone to quickly reduce the temperature differentials.

6. In a process for the treatment of ferrous metal bodies, the steps of rapidly cooling the object whereby marked temperature differentials are produced between portions of the body and then immersing the object while still hot in a liquid bath having a temperature not lower than the blue heat zone to quickly reduce the temperature differentials.

7. In a process for the treatment of ferrous metal bodies, the steps of rapidly cooling the bodies in an aqueous medium whereby a marked temperature differential is produced between the interior and exterior portions, and then immersing the bodies while still hot in a hot liquid metal to quickly reduce the temperature differentials.

8. In a process for the treatment of ferrous metal bodies, the steps of rapidly cooling at least a portion of the body through the

critical range and thereby producing marked temperature differentials between different portions of the body, and then immersing the body while still hot in a salt bath having a temperature not lower than the blue heat zone to quickly reduce the temperature differentials.

5. In a process for the treatment of rails, the steps of rapidly cooling a rail and then, 16 while the innermost portions of the head of the rail are still above the blue heat zone, immersing the rail in a molten bath of lead to quickly reduce the temperature differentials.

6. In testimony whereof I hereunto affix my 15 signature.

EDWARD F. KENNEY.

20

25

30

35

40

45

50

55

60

65